

## UNITED STATES PATENT OFFICE

2,061,328

## ART OF LUBRICATION

William B. D. Penniman, Baltimore, Md.

No Drawing. Application July 23, 1934,  
Serial No. 736,612

9 Claims. (Cl. 87—9)

This invention relates to lubricants, and their utilization, as well as to methods of making such lubricants.

From a broad and general consideration, the lubrication of machines and machine elements, including for example bearings, gears, cylinders, etc., is dependent upon a number of factors including the mechanical construction and speed and load on the bearing surfaces to be lubricated, on the supply of lubricant, and on the kind and properties of the lubricants. The present invention is particularly concerned with the kind and properties of lubricants used in lubrication.

Consideration of the nature of the lubricant employed, requires a consideration of the widely varying conditions under which lubricants may be used. Such conditions under which two surfaces pass over one another vary from the high speed and high temperatures involved in internal combustion engines to the relatively low speed and low temperatures present in swivel plates, for example, of a railroad turntable.

Generally the lubrication of any given bearing to take a typical case, is dependent upon first, the supply of lubricant, second the viscosity of the lubricant, and third, the "oiliness" of the lubricant.

The lubricants generally employed, are of hydrocarbon type, petroleum oil and oils of related nature, such as those obtained from shale and coal by distillation, being the main source of supply of lubricants the world over. While such petroleum oils and related substances vary considerably among themselves, in general it has been noted that as the viscosity of the oil increases, the oiliness also increases. Consequently, it had become the standardized practice to specify the lubricant in terms of its viscosity which was readily determined, thereby more or less loosely fixing the oiliness property desired. As a result in using these mineral and related oils, in order to obtain the required degree of oiliness, it was necessary to use oils of relatively high viscosity.

The practice in the prior art is well illustrated by referring to standard reference works, such as that of T. C. Thompson who lists eighteen oils

with viscosity numbers of 1 to 18, and ranging in viscosity as follows:

| Viscosity Nos. | Saybolt seconds |         |         | 5  |
|----------------|-----------------|---------|---------|----|
|                | 100° F.         | 130° F. | 212° F. |    |
| 1.             | 65              | 45      | 29      |    |
| 2.             | 80              | 50      | 31      |    |
| 3.             | 95              | 60      | 32      | 10 |
| 4.             | 125             | 70      | 34      |    |
| 5.             | 160             | 81      | 36      |    |
| 6.             | 180             | 86      | 38      |    |
| 7.             | 240             | 115     | 43      |    |
| 8.             | 350             | 160     | 50      |    |
| 9.             | 500             | 230     | 55      |    |
| 10.            | 700             | 320     | 65      | 15 |
| 11.            |                 |         | 80      |    |
| 12.            | 1400            | 470     | 90      |    |
| 13.            | 1800            | 600     | 100     |    |
| 14.            |                 |         | 130     |    |
| 15.            |                 |         | 165     |    |
| 16.            |                 |         | 190     |    |
| 17.            |                 |         | 700     |    |
| 18.            |                 |         | 1400    | 20 |

Under this designation of oils as given by Thompson in the work referred to, oils with the viscosity numbers 1 to 5, inclusive, are the so-called spindle oils. They do not generally enter into the lubrication program of the prior art, and are not generally considered in such program. Oils in the range from viscosity numbers 7 to 9, that is oils having viscosities of from 240 to about 600 Saybolt seconds at 100° F. are the oils generally used in the prior art in connection with the lubrication of the journals and axles of railway rolling stock, such as those of steam and electric street railways.

As further illustrating the prior art reliance on the use of heavy or viscous lubricating oils, reference may be made to the specifications set out in Technical Paper No. 323A of the Bureau of Mines, United States Government, and entitled "United States Government Specifications for Lubricants and Liquid Fuels and Methods of Testing". On page 28 of this paper, the names and grades of the various lubricants are set forth. But in this paper, the lightest grade of oil suggested for lubrication is a so-called "Class A, Extra Light" having a viscosity of about 135° at 100° F.; while on page 9 of this paper the whole Class A embracing oils with viscosities of from 135 to 360° is given as used only for very light machinery. So that under these specifications, 50

the use of an oil of a viscosity below 135" at 100° F. is not contemplated for any purpose, and those in the range of 135 to 360" are used for very light machinery only.

- 5 The statements in this paper of the Bureau of Mines exemplifies the attitude of the entire industry where the use of relatively heavy lubricants is universally followed, particularly in connection with the lubrication of heavy machinery.
- 10 As exemplary of this prior art practice, reference may be made to the practice in connection with the lubrication of internal combustion engines, such as those employed in automobiles. It is customary in that art where the speed and
- 15 load are high, to mix with the lubricating oil, large percentages of cylinder stock, or other very heavy oils in order to obtain the desired adhesiveness. And so much is this the custom in this field that petroleum lubricating oils are generally sold on the basis of their viscosity only, whereby the adhesiveness is in this way secured to a greater or lesser extent.

This prior art practice is further illustrated by reference to the lubrication of street railway journals or axles, particularly of those of steam and electric street railways. In this field, oils of the viscosity of from 250 to 600" Saybolt at 100° F. are generally used. A further consideration in this and other analogous cases was the fact that the operating temperatures of the bearing or related mechanism under certain circumstances might be about 100° F. or even higher; with the result that the viscosity of the lubricant was chosen from the standpoint of such higher temperature operation. The variation in viscosity of these prior art lubricants, which change in temperature over the usual operating range, was quite marked, so that when the lubricant operated at the higher temperatures, it necessarily possessed a much higher viscosity at the lower temperatures. And in fact in many instances, these lubricants in order to give the requisite viscosity at the higher temperatures were actually solids at temperatures such as those frequently reached in this climate during the winter season.

The choice of heavy or viscous materials in accordance with such prior art practices, in order to secure adequate adhesiveness, result in a tremendous loss of power due to the internal friction of the lubricants. But these losses in power were either not recognized or appreciated in the prior art, or else were accepted as unavoidable.

Among the objects of the present invention is the production and use of lubricants of the lowest possible viscosity consistent with the heat conditions under which they are to be used.

A further object of the invention is the utilization with such low viscosity lubricants of components added thereto for increasing the oiliness or adhesiveness of the low viscosity materials.

Still further objects of the present invention include the incorporation into the low viscosity lubricants of layer-forming components to insure the production of adequate lubricating oil films between the surfaces to be lubricated.

Other and further objects and advantages of the invention will appear from the more detailed description set forth below, it being understood however that various changes within the scope of this invention may be made by those skilled in the art without departing from the spirit and scope of this invention as herein disclosed.

Accordingly in accordance with the present invention, the lubricant is preferably based on the utilization of hydrocarbon stock, such as that derived from petroleum and related oils, which hydrocarbon stock is of the lowest possible viscosity consistent with the heat conditions under which the lubricant is to be used, far lower than that normally employed for the lubrication of heavy machinery. While the lowest possible viscosity material is thus chosen, regard must be had for the flash point, fire test, and similar factors, where those factors are important. For example, in connection with the lubrication of internal combustion engines, the viscosity of the hydrocarbon stock would have to be higher in order to secure the necessary flash point, etc., than would the lubricant used for the lubrication of an ice machine, where such factors would be of little importance. In any event, in accordance with the present invention, the oil of lowest possible viscosity is preferably chosen, having in mind the heat conditions under which it is to be used. The use of these low viscosity oils is advantageous, and particularly when full fluid or viscous friction is to be utilized, as the amount of friction under these conditions is dependent upon the viscosity only, and the lower the viscosity, the more economical is the lubrication. Further, the power losses due to the prior art use of heavy lubricants is thus avoided.

Now while the viscosity should be as low as possible, the adhesive property should be as high as possible in any of these given lubricants. When a bearing, for example, comes to a stop, or when for any other reason, the so-called greasy layer has to take up the work for a short time, the lubricant must have the power of forming a greasy layer sufficiently thick to act as a cushion between the metallic surfaces, and must be sufficiently adherent to remain on the surfaces of the metals under severe conditions of service. For some years, the property of oiliness of ordinary petroleum oil was improved by the addition of saponifiable oil or fatty acids of saponifiable oil.

The principle on which an oily or greasy agent is added to the petroleum or other stock is based upon the fact that bearing surfaces by their surface energy preferentially attract from the lubricant to themselves certain portions of the lubricant, and it has been found that the first layer of molecules so attracted may be held to the varying surfaces with great tenacity. This initial layer upon the surface is almost infinitely thin, and though useful is not sufficiently thick to protect the metallic or other surface against rupture of this thin oily film; which rupture though at portions only of the thin oily film, give rise to undue friction and possible injury to the bearing surfaces. Further, the building up of the first layer involves a time interval that must be considered, and when the amount of material such as fatty acid, which is readily absorbed by the bearing surface is present in the lubricant in small proportion only, the disturbance created by the relative motion of the journal and bearing or other parts being lubricated may interfere with the formation or reformation of the first layer sufficiently to cause injury during the interval of its formation.

Consequently to increase the oiliness or adhesiveness of the low viscosity stock which is the basic component of lubricants in accordance with the present invention, these components are added which may be termed as a class, polar bodies. Such added components for increasing the oil-

ness or adhesiveness of the lubricant stock are compounds or mixtures of compounds containing a substituent group for which the surface forces of the metals have a particular attraction.

Now while as pointed out above, there is included with the low viscosity hydrocarbon stock, added components giving oiliness or greasiness properties, which components are used desirably in substantial amounts and will be exemplified below from a wide field of choice, such polar bodies form only a relatively thin layer immediately adjacent to the metal surfaces, and it is desirable to place in the stock a substance or substances to build up the initially formed thin layer into a relatively thick one to protect the surface against any possible injury during the interval when this primary layer is being formed, or at any time that this primary layer becomes ruptured. This may be done, for example, by adding substances which are attracted preferentially to the adsorbed primary layer or readily commingled with the substance or substances forming the primary layer. These additional layers, which are built up by such added substances may be called mush layers, and a lubricant which has the property of building up these so-called mush layers may be referred to as one having the property of mushiness. These mush layers are more resistant the closer they are to the initial or adsorbed layer, and fade off gradually into the average composition of the lubricant. The total depth or thickness of the mush layer can be made within reason as great as requisite.

Accordingly the most desirable form of lubricant will be a compounded oil that possesses low viscosity, high adhesiveness, and the ability to build up mush or protecting layers.

In accordance with the present invention, there is accordingly used lubricating oil stock whether derived from petroleum or the products of distillation of coal and shale, which oil stock has the lowest possible viscosity for the conditions under which the machine operates; that is the lowest viscosity that is obtainable with requisite flash point to withstand the temperature prevalent during use. And this applies whether the lubricant stock is derived from a straight paraffin stock, or from a so-called asphaltic or semi-asphaltic base oil. For cold conditions or climates the non-paraffin base oils have lower freezing points than the paraffin base oils, and are in general more desirable for this reason.

Low viscosity material for use in the lubrication of heavy machinery, and having the requisite flash point, etc. was not available on the open market in spite of the wide variety of products produced by the various oil companies and refineries. So that such low viscosity material had to be made for the first time and methods were developed for its production.

For example, a desirable stock may be made by distilling off about 75% of the lighter material from kerosene oil, and using the remainder in the still as "stock" for the preparation of the finished lubricant. As a result of such distillation, the residue in the still is a product of requisite fire point and cold test with much lower viscosity than that commercially available prior to the present invention. Products are thus produced having a viscosity of approximately from 150 to 160" at 100° F. as an upper limit.

Similar products of low viscosity may be prepared from the distillate of petroleum coal tar or shale oil in the range from which burning oils and not lubricants are generally prepared. These

distillates I use as a base stock for special lubricants, as they can be secured with sufficiently high resistance to volatilization and low viscosity and are relatively slow to oxidize or sludge.

Thus a specific product obtained by distilling off 75% of ordinary coal oil tested as follows:

|                           |                     |    |
|---------------------------|---------------------|----|
| Specific gravity at       | 60° F., 38.5 Bé.    | 10 |
| Flash point               | 240° F.             |    |
| Fire point                | 275° F.             |    |
| Viscosity at              | 40° F., 74" (S. U.) | 10 |
| Viscosity at              | 60° F., 56"         |    |
| Viscosity at              | 80° F., 45"         |    |
| Viscosity at              | 100° F., 40"        |    |
| Viscosity at              | 210° F., 31"        | 15 |
| Cold test below           | 0° F.               |    |
| Total saponifiable matter | 11.3%               |    |
| Free fatty acids          | 1.2%                |    |

Similar products as to viscosity may be prepared from any of the other distillates of light boiling points, petroleum, coal tar or shale oil.

In general it may be stated that where flash point is an important consideration, the viscosity of the hydrocarbon stock should not be so low that the product has a flash point of below about 225 to 230° F.; but as noted above, in connection with the more general considerations there given, these factors are variable depending upon the use to which the lubricant is to be put.

As indicative further of oils that may be used, products having the following characteristics may be noted:

|                           | I    | II   | III | 35 |
|---------------------------|------|------|-----|----|
| Gravity at 60° F.         | 24.8 | 24.8 |     |    |
| Flash point 0° F.         | 290. | 280. | 235 |    |
| Fire point 0° F.          | 340. | 340. | 265 |    |
| Viscosity at 100° F. ("") | 72   | 60.  | 44  |    |

The products such as those indicated above are particularly desirably used in connection with the present invention. Further with materials having such low viscosities as those indicated under the third example given immediately above, the material exhibits a substantially uniform viscosity over the usual temperature scale prevailing under conditions of use, and this substantial uniformity of viscosity over the usual working scale is particularly desirable in the lubrication program.

While as noted above, the upper limit of viscosity of the hydrocarbon stock is preferably about 150 or 160" Saybolt at 100° F., there is no lower limit as to viscosity that can be employed, but oils running from 65" down as low as can be obtained, as probably around 35", may be utilized in accordance with the present invention.

The utilization of this low viscosity material as discussed above in the production of lubricants will, of course, depend on the particular machinery which is to be lubricated. In all cases, however, the lubricant produced in accordance with the present invention will utilize a hydrocarbon stock that is far lower in viscosity than was normally considered adequate for such work in the prior art. In general, it will be noted in accordance with the considerations given above that the spindle oils, as for example the first five oils of the Thompson tabulation above given, and having a viscosity at 100° F. of between 65 and 160" Saybolt, were limited for use on textile spindles where the load is practically zero and the speed is rather high. Such spindle oils have

never been used in the lubrication of heavy machinery.

On the other hand, in accordance with the present invention, such low viscosity materials of the order of spindle oils, compounded in accordance with the present invention to give them requisite oiliness and mushiness, but still retaining their relatively low viscosities, are used for heavy machine lubrication.

Thus for the lubrication of street railway journals where the prior art required hydrocarbon stock having a viscosity of between 250 to 600" Saybolt at 100° F., in accordance with the present invention, a hydrocarbon stock will be employed having a viscosity less than 150-160" Saybolt at 100° F., and preferably with a viscosity of only about 100" Saybolt at 100° F.

But the invention is not limited to the utilization of such low viscosity materials in connection with the lubrication of heavy machinery, since the invention may also be utilized in connection with improvements of the lubricants used for lubrication of spindles. Whereas in the prior art, as illustrated in the Thompson tabulation, the spindle oils employed have viscosities of about 65 to 160" Saybolt at 100° F., in accordance with the present invention it will be permissible to use oils of a much lower viscosity, such as oils from 35 to 65" Saybolt at 100° F. when compounded with ingredients for increasing oiliness or adhesiveness, and/or materials which secure the protecting film referred to above.

Referring to the character of lubricants for use in internal combustion engines, such as automobile engines particularly, several specific considerations may be noted. The useful work, i. e. energy delivered to the driving wheels of an automobile, is only about 18% of the total power developed. Most of the energy loss is in the cooling water and waste gas which together total about

the friction is full "fluid", but the character and thickness of the mush layer is evidently important. Other characteristics enter that need not be taken up in detail, such as character of decomposition under heat, kind of carbon formed in the cylinder, gumming deposits in the piston rings and valves, ease of combustion of residual deposits on cylinder walls, etc.

In general (for there are a few exceptions) the same oil is used for the lubrication of cylinders and bearings of the engine, as in an automobile. These latter operate, however, under very different conditions: first, the temperature is much lower during the major time of operation; second, the oil feed is superabundant; and third, the load on different parts of the bearing varies continually as the engine operates. The lubrication evidently is almost entirely of the "full fluid" type, and where an oil of the lowest possible viscosity is used economy is evident, but sufficient film-forming power to withstand "squeezing" when the maximum load is applied is also necessary. This maximum evidently occurs during the time when the fuel is burnt (exploded) in the cylinder. Throughout the whole mechanism the heavy load is applied only 25% of the time to the cylinders or bearings (except those which carry the crank shaft on which the load in pulsating but more nearly continuous).

Comparing now the viscosity of the oils in general use in internal combustion engines with those which will be employed in accordance with the present invention, the following table is given—it being understood, of course, that in all of the oils designated as "Penniman oils" or "Compounded oils made in accordance with the present invention", they will include the materials necessary to build up the required protecting film, or to give the oiliness and adhesiveness characteristics required in such compounded oils:

|                                                              | Extra light | Light       | Medium     | Heavy       | Extra heavy<br>Diesel engine |
|--------------------------------------------------------------|-------------|-------------|------------|-------------|------------------------------|
| Viscosity at 100° (S. U.)                                    |             |             |            |             |                              |
| Kinematic viscosity                                          | 175<br>.38  | 250<br>.51  | 400<br>.83 | 650<br>1.35 | 1000<br>2.05                 |
| Penniman's Oil (S. U.)                                       |             |             |            |             |                              |
| Viscosity at 100° F.                                         | 38<br>.1313 | 60<br>.0942 | 72<br>.12  | 100<br>.20  | 200<br>.4                    |
| Kinematic viscosity                                          |             |             |            |             |                              |
| Power Saving if the friction were "full<br>fluid" at 100° F. | 91%         | 81%         | 85%        | 85%         | 80%                          |

70% of the total energy. The engine friction loss is about 5.6% of the total energy and transmission friction losses are about 2.9% of the total energy developed. Disregarding the other losses, therefore, it is evident that if friction could be done away with entirely—which of course is impossible—the useful work done would be raised from 18 to 26.5%, or an increase of useful work of 47%.

The character of the lubricants used in internal combustion engines is of particular interest and importance. The machine in such cases from the lubrication standpoint may be considered from two standpoints—that of (a) the bearings and (b) the pistons. The piston lubrication requires an oil that will withstand a relatively high temperature, and it must adhere to the surfaces of the cylinder and piston to secure a reasonable reduction of friction. The viscosity of the oil at temperatures varying from, say, 200° F. to 300° F. is evidently important as much of

The above figures of percentage saving are at 55 100° F. and change inversely with the temperature, for as the temperature increases the relative differences in viscosity become smaller, the film forming qualities also decrease.

Lubricants used in the transmission are in general the greases or heavy residual oils. The temperatures are comparatively low and the difference between them and that of the surrounding air is due to friction only. On account of the way that gears engage, a small area at any one time is subject to a rolling squeezing action that renders an adherent mushy film advisable. The squeezing out of a high viscosity lubricant immediately before the high pressure moment is reached is evidently a waste of power, which can only be lessened by using an oil of low viscosity, but this oil to be serviceable must have high "mushiness", as well as the property commonly called "oiliness". The prior art types of lubricants used have had viscosities of about 800" Saybolt 75

universal, or slightly below that figure, which figure represents the minimum or lightest oil used. In accordance with the present invention, however, the compounded oils having viscosities 5 in the range of that given above for lubrication of internal combustion engines and running up to a viscosity of about 200 to 250 will be utilized under the practice of the present invention.

The practical effect in the operation of a motor 10 car, for example, by utilizing the lubricants of the present invention is a saving in motor fuel and/or an increase in speed and power for the same consumption of fuel. These savings often amount to 25% or more after the engine has heated up 15 to its maximum operating temperature, and are, of course, greater until a heat balance is reached, and in very cold weather when an economical heat balance is never reached, the economy effected is much greater.

20 While in some cases, as in turbines, and similar machinery where the lubricant is pumped about a bearing by external means, the low viscosity stock may be utilized by itself for lubrication, its use in the ordinary bearing where no pumping 25 action is present aside from that produced by the rotation of the bearing itself or the journal, is desirably carried out in conjunction with the added ingredient for improving the properties as to oiliness and mushiness.

20 The low viscosity oils, particularly of hydrocarbon stock character, are thus desirably compounded with added ingredients for increasing their oiliness or adhesiveness, and their capacity to build up the so-called mush or protecting 30 layers. As exemplary of the polar compounds that may be employed for increasing the oiliness and adhesiveness of these compositions, there may be mentioned fatty acids, particularly the higher fatty acids, such as for example, the 35 fatty acids of castor oil, etc. The higher the fatty acid the better appears to be its effect, and the presence of additional groups such as the hydroxyl group in the molecule with the carboxyl group appears to yield a better lubricant. The 40 polar bodies are not limited to the fatty acids, but the non-fatty acid polar bodies, compounds or materials may be employed. The higher alcohols and ketones are advantageous and work almost as well as the fatty acids. Sulphides and 45 some of the metallic salts are also efficient, though in general due to the ready availability of the fatty acids and their cheapness, they are more desirably employed. The higher alcohols and ketones may be readily obtained, for example 50 from the oxidation products obtained during the air blowing of petroleum and related materials, particularly under pressure and at elevated temperatures, or from the residues remaining in the 55 still during such air blowing processes. The sulphides may be prepared by direct treatment of petroleum oil with sulphur, the products being somewhat complex, but the polar bodies appear and their effect is available.

60 In those cases where the use of fatty acids may be objectionable due to the possible effect of such acids on the metal of the bearing or journal, the polar body may be chosen with such considerations in mind to avoid the presence of free acid 65 groups of damaging characteristics.

70 The following method of preparing sulphur compounds for admixture with the oils in accordance with the present invention may be utilized where the oil may reach temperatures 75 above 175° F. Tallow oil is heated with 15% of

sulphur while agitating, for about two hours at 350° F. until the initial reactions are completed. The reactions taking place are quite active and a good deal of the sulphur is lost by volatilization. The temperature is then raised to 400° F. or higher and kept at this temperature until the resulting composition will no longer darken a copper strip brought in contact with it. The sulphur base compound thus obtained is only slightly soluble in petroleum, and it is desirably utilized by compounding with from 50 to 75% of a saponifiable oil. From such resulting composition containing the saponifiable oil, from 2 to 15% of such composition is used in the petroleum or other hydrocarbon oils of the viscosities given herein.

10 The sulphur base compound acts as a polar compound and adheres tenaciously to the metallic surfaces of the metals, dragging with it considerable quantities of the saponifiable oil, and perhaps some of the constituents of the petroleum. 15 Both adherence and thickness of film are secured in this way.

For the building up of the mush or protecting layers, various substances are available. The best effect is obtained with a material that is 20 soluble in the polar body and substantially insoluble in the petroleum oil or hydrocarbon stock, so that when a portion of the fatty acid or other polar body adheres to the metal surface to form the primary layer, a very considerable quantity 25 of the mush substance is withdrawn, and a thicker and more coherent mush layer built up. Saponifiable oils or fats that contain some fatty acid to act as the polar body serve in this connection. If the amount of fatty acid is small, the polar fat- 30 35 acid will be withdrawn, and will act to take up but a comparatively small quantity of the mush ingredient, namely the neutral glycerides or fats, and a comparatively thin and soft coating results. The presence of comparatively large 40 quantities of substances more attracted to the polar body will assist in building up a better mush layer.

The ketones, and particularly complex mixtures of ketones as may be obtained from the heat 45 treatment of the higher fatty acids may desirably be utilized as "mushiness" ingredients, although they also exhibit "oiliness" characteristics to a considerable extent. They may be prepared, for example, from the fatty acids, using iron as a 50 catalyst, by heating until the condensation is effected, or the heating can be stopped when only a portion of the acid or acids have been converted into ketones. Since the pure ketones are 55 not very soluble in petroleum oil, it is generally better to use a mixture of fatty acids, such as are readily obtainable from cocoanut oil. When using the ketones and other substances formed in the way indicated, it is generally advisable to blend them with tallow, lard oil or other similar 60 materials to improve the mushiness and for economical reasons, and to use such compositions of such ketones with tallow, lard oil, etc. for addition to the hydrocarbon stock material.

65 As a good example of materials to be used in building up the mush layer while also exhibiting the necessary polar properties, castor oil dissolved in oleic acid will serve, the castor oil being substantially insoluble in the petroleum oil stock used. Thus 2 parts of castor oil to 1 part of oleic 70 acid may be employed. The oleic acid acting as the polar body carries down with it large quantities of the castor oil and the mush layer consists largely of oleic acid and castor oil. This artificial or synthetic composition builds up a better 75

layer than does an ordinary animal oil consisting of a mixture of some free acid and natural glycerides, although the latter may be employed.

Insofar as the formation of the mush layer 5 is concerned, it does not appear to be material whether the substances are in solution or in colloidal condition, and either or both are available for use in accordance with the present invention. Any method by which molecular attraction, i. e., the clinging together of molecules by either known chemical attraction or residual chemical forces, may be made use of. It is well known that substances used in lubrication build up a surface film on the metallic surface of considerable tenacity. Other substances may also 10 form or build up such films, but they are not of value as lubricants. In those cases where the fatty acids are objectionable in the lubricant, the substituted ammonias that have little value as 15 lubricants but build up films on the surface can be used. If there is also added some material of high lubrication power that is selectively absorbed by the substituted ammonia, or which forms molecular aggregates with it, a satisfactory result 20 is secured. In the lubrication of internal combustion engines, where high temperatures prevail, the avoidance of such acidity is desirable. In such cases, there may be employed a mixture, for example, of diphenylamine and tallow oil (the latter containing little or no free acid). Good results 25 are obtained when only 5% of this mixture is added to the selected petroleum stock.

Soaps which form an emulsion with the petroleum stock, or which are soluble in the 30 petroleum stock can also be used. For example, soaps with petroleum stock, particularly the soda and lime soaps that are present as colloids.

The soaps that go into solution include lead 35 oleate, copper oleate, and the oleates of the heavy metals generally, the alkalies and alkaline earth metals forming colloids. As apparently soluble compounds, there may be mentioned copper oleate, zinc oleate and sodium sulphur oleate, while ordinary calcium and sodium oleate when used 40 are present as colloids.

Animal oils, such as lard oil, may be used in amounts as exemplified by 10%, but other oils, such as tallow oil which contains some free acid 45 is preferable to lard oil, and castor oil when in solution as illustrated above is superior to either lard oil or tallow oil.

In some cases, the body added to improve the mushiness characteristic may at the same time possess a polar property, so that in this way two 50 purposes can be secured at the same time. This is particularly true of some of the sulphur compounds in the nature of sulphides illustrated above, as well as with the class of compounds known as sulphonic acids. As exemplary of the 55 sulphonic acids that may be used for this purpose, the following is given.

Sulphonic acids derived from the treatment of 60 unsaturated petroleum compounds, that is to say those obtained from the residue of the purification of ordinary petroleum oil by treatment with sulphuric acid are available for present purposes. These sulphonic bodies are of indefinite chemical 65 composition. The sulphonic acid group  $\text{HSO}_3$  in these bodies acts as the polar body. Sulphonic acids can also be prepared and used which are 70 dyestuff intermediates, and these compounds may be very complex or elaborate. The simple hydrocarbons and the more complex ring compounds including double and triple rings may 75 serve in this connection for the production of

these sulphonic derivatives. As an example of dyestuff intermediates utilizable in this connection mention may be made of the naphthol sulphonates.

These bodies which serve as both the polar and 5 mushiness ingredients may of course be used as the polar ingredient alone, and in general it has been found more desirable to use two separate ingredients for this purpose rather than to attempt to accomplish both ends with a single 10 substance.

Further it may be noted that when high temperatures avail in use, the oils have a tendency to oxidize rather readily with the formation of 15 gummy materials that are disadvantageous in practice. Some of the animal and vegetable oils and their derivatives used as the greasy or oiliness components, oxidize less readily than others, but all of them even when mixed with mineral 20 oils oxidize to a greater or lesser extent, and some like cottonseed oil and corn oil are seldom or never used either alone or mixed with mineral oil on account of this ease of oxidation. To prevent such oxidation, substances may be introduced 25 into the lubricant composition that lessen or prevent the oxidation of oil under given conditions of service, so that undesirable changes in the oil due to oxidation rendering them undesirable from many points of view are avoided or eliminated entirely. The use of anti-oxidants 30 evidently broadens the field in use of vegetable oils and mineral oils, as mineral oils also oxidize to a lesser extent than the vegetable and animal oils. The anti-oxidant may be any substance 35 that in a general sense reduces the effect of oxidation or air upon the lubricant. As such, there may be mentioned tetraethyl lead, phenol disulphide, amino and amide compounds, phenols, such as pyrogallol, hydroquinone, and other substances such as elementary sulphur, malachite 40 green. The amount of the anti-oxidant is varied according to the time at which the lubricant is to be used, and the conditions as to oxidation. At a very low temperature, the effect of the oxygen is very little feared, so that the amount of anti-45 oxidant used in such cases, may be as low as .1%. The dinaphthylamine is desirable, but tetraethyl lead has also proved to be moderately efficient.

The amounts of the components added to increase oiliness or adhesiveness, and to build up 50 the mush or protecting layers, may vary within substantial limits, such as up to 15%, although more than 10% will generally not be required. Lesser amounts can, of course, be utilized. The amounts of such added components should not 55 materially or substantially affect the viscosity of the hydrocarbon stock, or of the final composition, and at least should not carry the viscosity beyond the point desired for the particular purposes for which the lubricant is designed.

The following specific example of a lubricant 60 made in accordance with the present invention and utilized in connection with the lubrication of street railway journals, and which has proved particularly advantageous in such practice is given.

2 parts of castor oil are dissolved in commercial oleic acid, and the mixture heated to about 160° F. to insure solution. The resultant product is admixed or added to petroleum stock having the 70 characteristics set forth above, the castor oil, oleic acid mixture constituting 5% of the total admixture. When used at a relatively elevated temperature, 1 part of beta beta dinaphthylamine is added to the oil as an anti-oxidant; while 75

if the oil is to be used at normal temperatures 1 part of mono-methylaniline may be employed. An excellent product is thus secured.

Other types of compositions may be made by 5 adding 10% of lard oil, for example, to the hydrocarbon stock material described above and numbered I, II and III.

As exemplary of the phenomenal results flowing 10 from the present invention, attention may be called to the fact that it has been applied in the lubrication of a large railway system where about 30,000 bearings were under study. Whereas it has been the custom to use oils of viscosity of about 250" viscosity Saybolt on 15 such railway system prior to the development of the present invention, in accordance with the present invention, the lubrication of bearings on that street railway system is now being made with oils of a viscosity of 35" Saybolt at 20 100° F. Lubrication by means of these low viscosity oils in accordance with the present invention has resulted approximately in a reduction in power costs of about 20% annually.

Comparable results have been obtained in connection 25 with the lubrication of internal combustion engines, such as automobile engines. In one case, for example, utilizing a low viscosity oil lubricant in accordance with the present invention the horsepower developed was 17.4; as 30 compared with 14.2 utilizing the ordinary automobile oil of the prior art. And in addition, by the utilization of the low viscosity oil, not only was there the phenomenal increase in horsepower referred to above, but the gasoline 35 consumption was reduced about 33%, even though the horsepower developed was as markedly great as that noted above.

Having thus set forth my invention, I claim:

1. A method of lubricating internal combustion 40 engines such as automobile engines which comprises utilizing therein a lubricating oil containing a hydrocarbon oil having a viscosity within the range of 135 to 200" Saybolt at 100° F., and a component for increasing the oiliness of the composition but, not increasing the viscosity of the composition substantially beyond 200" Saybolt.

2. A method of lubricating internal combustion 50 engines such as automobile engines which comprises utilizing therein a lubricating oil containing a hydrocarbon oil having a viscosity within the range 135" to 250" Saybolt at 100° F., and substantially less than that normally used for lubrication of automobile engines, and a component for increasing the oiliness of the composition and a mushiness component, the oiliness and mushiness components not increasing the viscosity substantially beyond 250" Saybolt.

3. A lubricating oil for internal combustion 60 engines, said oil containing a hydrocarbon oil having a viscosity above 135" and below 250" Saybolt at 100° F. and a component for increasing the oiliness of the composition without sub-

stantially increasing the viscosity beyond 250" Saybolt.

4. A lubricating oil for internal combustion engines, said oil containing a hydrocarbon oil having a viscosity within the range 135" to 250" Saybolt, but substantially less than that normally used for lubrication of internal combustion engines, and a component for increasing the oiliness of the composition and a mushiness component, the oiliness and mushiness components not increasing the viscosity substantially beyond 250" Saybolt. 10

5. A lubricating oil for internal combustion engines, said oil containing a hydrocarbon oil having a viscosity within the range of 135 to 200" Saybolt at 100° F., and having a flash point not substantially below 225° F., and a component in an amount not exceeding 15% of the composition, for increasing the oiliness of the composition without substantially increasing the 20 viscosity beyond 200" Saybolt.

6. A lubricating oil for internal combustion engines, said oil containing a hydrocarbon oil having a viscosity within the range of 135 to 200" Saybolt at 100° F. but substantially less than that normally used for lubrication of internal combustion engines, a component for increasing the oiliness of the composition, and a mushiness component, the oiliness and mushiness components together not exceeding about 15% of the final composition and not increasing the viscosity substantially beyond 200" Saybolt. 25 30

7. A lubricating oil for internal combustion engines, said oil containing a hydrocarbon oil having a viscosity within the range of 135 to 200" Saybolt at 100° F. and a component including tallow oil and diphenylamine for increasing the oiliness of the composition without substantially increasing the viscosity beyond 200" Saybolt, the tallow oil and diphenylamine together constituting not substantially more than 5% of the composition. 40

8. A lubricating oil for internal combustion engines, said oil containing a hydrocarbon oil having a viscosity within the range of 135 to 200" Saybolt at 100° F., and a component for increasing the oiliness of the composition without substantially increasing the viscosity beyond 200" Saybolt, said component including sulphurized tallow oil and a saponifiable oil, the sulphurized tallow oil and saponifiable oil together constituting between 2 to 15% of the composition. 45 50

9. A lubricating oil for internal combustion engines, said oil containing a hydrocarbon oil having a viscosity within the range of 135 to 200" Saybolt at 100° F., and a component for increasing the oiliness of the composition without substantially increasing the viscosity beyond 200" Saybolt, said component including a saponifiable oil and ketone, the saponifiable oil and ketone constituting not substantially more than 15% of the composition. 55 60

WILLIAM B. D. PENNIMAN. 65